

[54] **FUNCTIONAL FLUID COMPOSITIONS**[75] Inventor: **Martin B. Sheratte, Reseda, Calif.**[73] Assignee: **McDonnell Douglas Corporation,**  
Long Beach, Calif.[22] Filed: **Mar. 11, 1974**[21] Appl. No.: **449,623****Related U.S. Application Data**

[63] Continuation-in-part of Ser. No. 230,131, Feb. 28, 1972.

[52] **U.S. Cl.** ..... 252/78; 252/49.8[51] **Int. Cl.<sup>2</sup>** ..... C09K 3/00; C10M 3/40[58] **Field of Search** ..... 252/78, 73, 49.8, 49.9[56] **References Cited****UNITED STATES PATENTS**

|           |         |               |              |
|-----------|---------|---------------|--------------|
| 2,549,270 | 4/1951  | Watson        | ..... 252/78 |
| 2,566,623 | 9/1951  | Moreton       | ..... 252/78 |
| 2,636,861 | 4/1953  | Watson        | ..... 252/78 |
| 2,659,699 | 11/1953 | George et al. | ..... 252/78 |

|           |        |                |                |
|-----------|--------|----------------|----------------|
| 2,687,377 | 8/1954 | Stewart et al. | ..... 252/78 X |
| 3,723,320 | 3/1973 | Herber et al.  | ..... 252/78   |
| 3,865,743 | 2/1975 | Sheratte       | ..... 252/78   |

*Primary Examiner*—Harris A. Pitlick*Attorney, Agent, or Firm*—Max Geldin; Max Geldin

## [57]

**ABSTRACT**

A functional fluid composition consisting essentially of (1) a phosphorus compound, preferably a phosphate ester containing at least two alkyl groups such as tri-n-butyl phosphate or di-n-butyl phenyl phosphate, alone or particularly in combination with a phosphate ester containing at least two aromatic groups, such as n-butyl diphenyl phosphate or tricresyl phosphate, and (2) a polyalkylene glycol material, e. g. a polypropylene glycol ether having a molecular weight ranging from about 600 to about 1200, and particularly a combination of at least two polyalkylene glycol materials, e.g. two polypropylene glycol ethers having substantially different molecular weights.

**15 Claims, No Drawings**

## FUNCTIONAL FLUID COMPOSITIONS

This application is a continuation-in-part of my co-pending application Ser. No. 230,131, filed Feb. 28, 1972.

This invention relates to functional fluid compositions having good fire resistance and desirable viscosity characteristics at both high and low temperature, and is especially directed to functional fluid compositions having the above-noted properties, particularly improved fire resistance and reduced deleterious effect on non-metallic materials, including reduced swelling effect on rubber, consisting essentially of a phosphorous compound, particularly certain phosphate esters and certain combinations of phosphate esters, and a polyalkylene glycol material, such as a polypropylene glycol ether of relatively low to medium molecular weight, and particularly combinations of certain polyalkylene glycol materials, the resulting functional fluids having the abovenoted desirable viscosity characteristics without requiring addition thereto of viscosity index improvers, such fluids also having improved thermal and hydrolytic stability and reduced density, as compared to conventional phosphate ester fluids, while otherwise retaining the desirable characteristics and advantages of conventional functional fluids containing chiefly a phosphate ester or mixtures thereof.

Many different types of materials are employed as functional fluids, and functional fluids are utilized in a wide variety of applications. Thus, such fluids have been utilized as electronic coolants, diffusion pump fluids, lubricants, damping fluid, power transmission and hydraulic fluids, heat transfer fluids and heat pump fluids. A particularly important application of such functional fluids has been their utilization as hydraulic fluids and lubricants in aircraft, requiring successful operation of such fluids over a wide temperature range, and fire resistant fluids.

Functional and hydraulic fluids employed in many industrial applications and particularly hydraulic fluids for aircraft must meet a number of important requirements. Thus, such hydraulic fluids particularly for aircraft use, should be operable over a wide temperature range, should have good stability at relatively high temperatures and preferably have lubricating characteristics. In addition to having the usual combination of properties making it a good lubricant or hydraulic fluid, such fluid should also have relatively low viscosity at extremely low temperatures and an adequately high viscosity at relatively high temperatures, and must have adequate stability at the high operating temperatures of use. Further, it is of importance that such fluids be compatible with and not adversely affect materials including metals and non-metals such as elastomeric or rubber seals of the system in which the fluid is employed. It is also important in aircraft hydraulic fluids and lubricants that such fluids have as high a fire resistance as possible to prevent ignition if such fluids are accidentally or as result of damage to the hydraulic system, sprayed onto or into contact with surfaces of materials of high temperature. Another important property for application of a hydraulic fluid in aircraft is the provision of a low density fluid to increase pay load.

Hydraulic fluids in commercial jet aircraft are exposed to temperatures ranging from below -40°F to over 200°F. Within these temperature extremes, it is necessary for the fluid to maintain a reasonably low

viscosity when cold, and yet not become too thin when hot. As a general rule, this means that the fluid preferably should have a viscosity of less than 4,200 cs. (centistokes) at -65°F, and maintain a viscosity preferably above 3.0 at 210°F.

Presently available commercial functional or hydraulic fluid base stocks do not possess these viscosity characteristics. Phosphate esters are among the most commonly employed base stocks, of which tributyl phosphate and dibutyl phenyl phosphate are widely used components. Both of the latter phosphates are too thin at high temperatures, and their use alone would result in rapid wear of moving parts. Other phosphate esters, such as tricresyl phosphate, for example, which provide the requisite high temperature viscosity become too thick to be useful at low temperatures. Even mixtures of various phosphate esters such as those noted above do not provide the required viscosity characteristics at both low and high temperatures. Accordingly, it has been the practice to achieve the required wide viscosity range required for aircraft hydraulic fluids by adding to a thin base stock, such as phosphate ester or mixtures thereof, a small proportion, e.g., up to 10%, of a polymeric material such as polyalkyl acrylates or methacrylates, whose solubility characteristics in the base stock are chosen so that the polymeric material thickens the fluid more at high temperatures than at low temperatures, and thus functions as a viscosity index (VI) improver.

However, the chief disadvantage of this method of viscosity improvement is that polymers of the type noted above are generally not stable to the shearing forces encountered in an aircraft hydraulic system, and during use, these large molecules are sheared down to smaller molecules which lose their ability to improve viscosity index. This means that the functional fluid loses viscosity in use and requires addition of polymer to the fluid and eventually, as the detritus from polymeric breakdown accumulates in the fluid and contaminates it, the fluid must be discarded. In addition, of course, employment of a viscosity index improver in the functional fluid, even in the minor amounts presently employed, substantially increases the cost of the fluid.

Polyalkylene glycol materials such as the co-polymer of ethylene oxide and 1,2-propylene oxide, having high molecular weight up to 15,000 to 20,000, have been employed as soluble organic polymeric thickeners in water based hydraulic fluids containing a water soluble glycol such as ethylene glycol, as the basic component, as disclosed in U.S. Pat. No. 2,602,780. However, such high molecular weight polyalkylene glycol materials have not heretofore been employed as a base stock component in essentially non-aqueous fire resistant phosphate ester based hydraulic fluids of the type according to the present invention.

U.S. Pat. No. 2,469,285 to White discloses a hydraulic pressure transmitting fluid such as a brake fluid, consisting essentially of tricresyl phosphate, along with solvents or diluents, such as a polymerized glycol and/or an aliphatic ether of a polyglycol, singly or in combination. However, such a fluid containing only tricresyl phosphate as the so-called lubricating base of the fluid, is too thick to be used as a hydraulic fluid for aircraft, at low temperatures ranging from -40°F to -65°F, even in the presence of the glycol materials employed as solvents or diluents in such fluid. Thus, as noted in the patent, the viscosity at -40°F. of represen-

tative examples of fluids according to this patent are about 9000 cs. and about 19,500 cs, which is substantially above the required viscosity for hydraulic fluids in commercial jet aircraft exposed to such low temperatures, such fluids preferably having a viscosity of less than 4200 cs. at the much lower temperature of -65°F. as noted above.

U.S. Pat. No. 2,801,968 to Furby et al. is directed to a jet turbine lubricant having as the main component a glycol ether employed in an amount of 90 to 98%, and which includes an antiwear additive in the form of a phosphate ester employed in minor proportions of only 0.5 to 5%. This composition is not a phosphate ester based hydraulic fluid, and it is noted that it is necessary to have the lubricant of this patent relatively thick because of the high operating temperatures of 550° to 650°F. of the lubricant, it being only necessary to be able to start the engine at low temperatures. Thus, in representative examples of this patent it is noted that at -65°F. the compositions of the patent have a viscosity ranging from almost 13,000 to 19,000 cs. Although such a high viscosity is permissible for use of the composition of the patent as a jet lubricant, that is to supply a film of lubricant to the moving parts of the jet engine, such high viscosities would render the composition of Furby et al. entirely unacceptable and inoperative to function as a hydraulic fluid continuously at such low temperatures, for example at -65°F. since as noted above a hydraulic fluid for successful operation of commercial jet aircraft at -65°F. preferably should have a viscosity of less than 4200 cs. at such temperature, while at the same time having sufficiently high viscosity at high temperatures also to continuously operate at the higher temperatures.

U.S. Pat. No. 2,839,468 to Stewart et al. has substantially the same disclosure as the above-noted Furby et al. U.S. Pat. No. 2,801,968.

U.S. Pat. No. 3,468,802 to Nail discloses hydraulic fluid compositions containing a phosphate ester as base stock component and discloses that various viscosity index improvers, including high molecular weight polyalkylene glycols, can be employed in minor proportion of from about 0.2 to about 12% by weight. It is noted that such high molecular polyalkylene glycol viscosity index improvers are characterized by having a high viscosity in the range of about 1400 to 23,000 cs. at 100°F.

U.S. Pat. No. 3,513,097 to Langenfeld discloses use of a wide variety of base stocks in functional fluid compositions, including esters and amides of phosphorus, among other types of base stocks. The patentee notes that the base stocks can also contain other fluids derived from coal products, for example alkylene oxide-type polymers, e.g. propylene oxide polymers. There is no disclosure or suggestion in this patent, however, of the combination of such alkylene oxide polymers with any specific types of base stock components, such as phosphate esters.

It is an object of this invention to provide a functional fluid which is particularly useful as an aircraft hydraulic fluid and which has requisite viscosity characteristics over a wide temperature range, and which has the advantage of not requiring incorporation of viscosity index improvers, while at the same time having other improved and other requisite properties for a good hydraulic fluid, including good fire resistance and low density, freedom from corrosivity and wear on metallic parts, and reduced deleterious effect on non-metallic

5 materials, e.g. reduced rubber swell, and having substantially reduced cost as compared to presently available aircraft hydraulic fluids, particularly those based essentially on phosphorous esters alone as the base stock component. Hence it is a particular object to replace such presently employed phosphorus ester base stock fluids, with functional fluids or blends containing base stock components or combinations thereof, in addition to phosphorus ester or phosphate components, which confer on the functional or hydraulic fluid, good viscosity and density characteristics, and other improved properties, while substantially reducing the cost of the fluid.

10 The above objects are achieved according to the present invention by the provision of a functional fluid, particularly valuable as a hydraulic fluid for aircraft, comprising basically a mixture of a phosphorus compound, particularly a phosphate ester containing at least two alkyl or alkoxyalkyl groups, hereinafter termed an "aliphatic" phosphate, and a polyalkylene glycol material, particularly a polypropylene glycol ether of relatively low to medium molecular weight. The phosphorus compound, e.g. phosphate ester, and polyalkylene glycol material are utilized preferably in the amounts or proportions set forth hereinafter, in order to obtain the desirable properties of the functional fluid noted above.

15 As a further feature of the invention it has been found that the incorporation ester containing at least two aromatic groups, e.g. diphenyl-n-butyl phosphate, hereinafter termed an "aromatic" phosphate, particularly in certain amounts noted below, in combination with a phosphate ester containing at least two alkyl groups, e.g. tributyl phosphate or di-n-butyl phenyl phosphate, the aliphatic phosphate, provides additional 20 advantages. In the first place, the presence of the phosphate ester containing at least two aromatic groups has been found unexpectedly to increase or improve the AIT (autoignition temperature) characteristics of the residing fluid or blend, over the fluid having only a phosphate ester or esters containing at least two alkyl groups, that is, the aliphatic phosphate. This advantage renders unnecessary the use of heavy metal, e.g. selenium or lead, or iodine, organic compounds as AIT 25 enhancers. This is particularly noticeable in blends containing an aliphatic phosphate and including polyglycol ethers such as polyethylene glycol or polypropylene glycol mono- or di-butyl ethers. Such blends generally exhibit AIT values below 700°F in the absence of either selenium additives, or aromatic phosphates.

30 Thus, in a functional fluid containing e.g. about 75% tributyl phosphate, and about 25% polyalkylene glycol material, by replacing a portion of such tributyl phosphate, e.g. 25% by weight of the fluid, with diphenyl octyl phosphate, the AIT of the resulting blend can be raised as much as 100°F or more over the fluid containing only the tributyl phosphate.

35 A further unexpected advantage of the presence of the aromatic phosphate together with the aliphatic phosphate is a marked decrease in the effect of such fluid blend on non-metallic materials, particularly elastomers such as rubber, as compared to fluids containing only an aliphatic phosphate or phosphates. Thus, the amount of rubber swell occurring on contact of such 40 fluid blend of aromatic and aliphatic phosphates with rubber materials such as rubber seals, is markedly reduced as contrasted to the amount of rubber swell produced by contact with fluids containing only ali-

phatic phosphates. Hence the presence of such aromatic phosphates in the above fluid blends causes a significant improvement in rubber compatibility. This is quite remarkable, since it is known, as pointed out in above U.S. Pat. No. 2,469,285 to White, that aromatic compounds are noted for their capacity to cause rubber swelling.

However, the presence of aromatic phosphates, such as tricresyl phosphate, in blends together with an aliphatic phosphate, such as tributyl phosphate causes the blend to be less responsive to the viscosity improving characteristics of the polyalkylene glycol component. As a further feature of the invention, it has been found advantageous to incorporate at least two different polyalkylene glycol components, that is at least two polyalkylene glycol materials, preferably at least two polyalkylene glycol ethers, that is, monoethers and/or diethers, having substantially different molecular weights, in the fluid or blend containing both the above-noted aromatic and aliphatic phosphates. The result is that the fluid blend can be more readily designed or tailored so that it has the above noted desirable low and high temperature and viscosity characteristics.

Thus, the functional fluids produced according to the invention can be blended as noted above to have a fire resistance greater than the fire resistance of presently employed commercially available hydraulic fluids, and at the same time to have suitably low viscosity at temperatures below -40°F, and down to -65°F, and suitably high viscosity at high temperature of 210°F, and above, and this can be accomplished without incorporating viscosity index improver. By avoiding the necessity for a viscosity index improver, the functional fluids of the invention do not suffer from the disadvantage noted above, namely, the deterioration of such polymeric additives used for viscosity improvement, and accumulation of molecular debris, leading to a shortening of the useful life of the fluid. Hence the functional fluids of the present invention have a longer period of usefulness, providing economic advantages including the avoidance of the high cost of the viscosity index improver and the employment of relatively low cost polyalkylene glycol ethers or diethers, in place of a substantial portion of the phosphate ester generally employed in presently available phosphate based aircraft hydraulic fluids.

Also, the functional fluid compositions and blends of the present invention have improved thermal and hydrolytic stability compared with the phosphate ester based fluids currently in use, contributing to a long useful life for the fluid. In addition, the functional fluids according to the present invention have low densities of the order of 1.0 or less, an important property for aircraft hydraulic fluids. The above advantages can be achieved while at the same time improving the flammability characteristics over phosphate ester-type hydraulic fluids currently in use. Also, the functional fluids according to the invention have freedom from corrosivity, wear and deterioration with respect to the metallic and non-metallic components, and the pumps of hydraulic fluid systems, which compare favorably with these characteristics for phosphate type base stock hydraulic fluids presently commercially employed.

Further, in addition to their valuable application as hydraulic fluids for aircraft hydraulic systems, the fluids according to the invention have important application as a hydraulic or functional fluid in industrial and marine fields, particularly in industrial turbine systems.

One of the essential components of the functional fluids according to the invention is a phosphorus compound selected from the group consisting of certain phosphate esters and amides of an acid of phosphorus, or mixtures thereof.

The basic aliphatic phosphate ester employed in the functional fluid according to the invention has the general formula:

10



15

where  $R_1$  and  $R_2$  each are alkyl, both straight chain and branched chain of from about 3 to about 10 carbon atoms such as n-propyl, n-butyl, n-amyl, n-hexyl, isopropyl, isobutyl, and the like, and alkoxyalkyl having from about 3 to about 8 carbon atoms such as methoxy methyl, methoxy ethyl, ethoxy ethyl, methoxy propyl, and the like, and  $R_3$  can be alkyl or alkoxyalkyl as defined above, or aryl such as phenyl and naphthyl, alkaryl such as cresyl, xylyl, ethyl phenyl, propyl phenyl, isopropyl phenyl, and the like, said aryl and alkaryl radicals preferably containing from 6 to about 8 carbon atoms.

20

Examples of such aliphatic phosphates are the trialkyl phosphates having alkyl groups which are either straight chain or branched chain with from about 3 to about 10 carbon atoms, such as n-propyl n-butyl, n-amyl and n-hexyl, particularly tri-n-butyl phosphate, tri(2-ethyl hexyl) phosphate and triisononyl phosphate, the straight chain alkyl groups preferably containing from 4 to 6 carbon atoms.

25

Other examples of such aliphatic phosphate esters are the dialkyl aryl phosphates in which the alkyl groups are either straight chain or branched chain and contain from about 3 to about 10 carbon atoms, such as n-propyl, n-butyl, n-amyl, n-hexyl, isopropyl, isobutyl, isoamyl, and the aryl radicals have from 6 to 8 carbon atoms and can be phenyl, cresyl or xylyl, particularly dialkyl phenyl phosphates including dibutyl phenyl phosphate, butyl amyl phenyl phosphate, butyl hexyl phenyl phosphate, butyl heptyl phenyl phosphate, butyl octyl phenyl phosphate, diethyl phenyl phosphate, amyl hexyl phenyl phosphate, amyl heptyl phenyl phosphate, and dihexyl phenyl phosphate.

30

In the above-noted preferred embodiment, the basic phosphate ester also includes an aromatic phosphate in combination with the above aliphatic phosphate. Such aromatic phosphate has the general formula:

35



40

where  $R_4$  and  $R_5$  are each aryl or alkaryl as defined above, and  $R_6$  can be aryl or aralkyl, or alkyl or alkoxyalkyl, as defined above, except that such alkyl can contain from about 3 to about 20 carbon atoms, as illustrated below.

45

Examples of such aromatic phosphates are triaryl phosphates in which the aryl radicals of such phosphates have from 6 to 8 carbon atoms, that is, may be phenyl, cresyl or xylyl, and in which the total number of carbon atoms in all three of the aryl radicals is from 18 to 24, and preferably wherein the three radicals include at least one cresyl or xylyl radical. Examples of such phosphates include triphenyl, tricresyl, trixylyl, phenyl

dicresyl, and cresyl diphenyl phosphates.

Examples of other phosphates also termed herein aromatic phosphates are alkyl diaryl phosphates in which the aryl radicals of such phosphates may have from 6 to 8 carbon atoms and may be phenyl, cresyl or xylol, and the alkyl radical may have from about 3 to about 20 carbon atoms, examples of which are given above. Examples of the alkyl diaryl phosphates include butyl diphenyl, amyl diphenyl, hexyl diphenyl, heptyl diphenyl, octyl diphenyl, 6-methyl heptyl diphenyl, 2-ethylhexyl diphenyl, decyl diphenyl, decyl dicresyl, tridecyl diphenyl, butyl phenyl cresyl, amyl phenyl xylol, and butyl dicresyl phosphates.

The above aliphatic and aromatic phosphate esters which can be employed generally are normally liquid between about -65°F and 210°F, except for triphenyl phosphate. Preferably, the abovenoted trialkyl phosphates such as tributyl phosphate or tri-n-hexyl phosphate are employed as the basic aliphatic phosphate, as such phosphates are particularly effective in achieving low viscosity at low temperature. However, the abovenoted dialkyl aryl phosphates such as dibutyl phenyl phosphate, also can be employed as the aliphatic phosphate, and such phosphate can be employed in combination with a trialkyl phosphate such as tributyl phosphate.

The aromatic phosphate preferably employed in combination with the basic aliphatic phosphate component in formulating the above-noted blends, are triaryl phosphates as illustrated above, e.g. tricresyl phosphate, particularly in combination with the abovenoted trialkyl phosphates, e.g. tributyl phosphate. However, the above-noted alkyl diaryl phosphate such as butyl diphenyl phosphate or octyl diphenyl phosphate or tridecyl diphenyl phosphate also can be employed, particularly in combination with the abovenoted trialkyl phosphate. Mixtures of aromatic phosphates also can be employed as the aromatic phosphate ester component.

Further, a mixture of three of the above aliphatic and aromatic phosphates can be used, e.g. a mixture of dibutyl phenyl, tributyl and triphenyl phosphates, or a mixture of tributyl, trihexyl and butyl diphenyl phosphates. Since triphenyl phosphate is a solid at ambient temperature, it is generally employed in combination with a liquid aliphatic phosphate in sufficient amount to maintain the combination liquid over the desired temperature range of operation of the fluid.

Another class of phosphorus compounds which can be employed as a base stock component according to the invention are the amides of acids of phosphorus, e.g., amido phosphates, including the mono-, di- and triamides of an acid of phosphorus, an example of which is phenyl N-methyl-N-n-butyl-N'-methyl-N'-n-butyl phosphorodiamide. Additional examples are m-cresyl-p-cresyl -N,N-dimethylphosphoroamidate, di-m-cresyl-N,N-dimethyl-phosphoroamidate, di-p-cresyl-N,N-dimethyl phosphoroamidate, phenyl-N,N-dimethyl-N',N'-dimethylphosphorodiamide, N-methyl-N-butyl-N'-N''-tetramethylphosphorotriamide, N,N'-di-n-propyl-N''-dimethylphosphorotriamide.

The second essential component of the functional fluid according to the invention is a polyalkylene glycol material. The polyalkylene glycol materials employed are compatible with the above-noted phosphorus compounds, particularly the phosphate esters.

Although polyalkylene glycols, e.g. polypropylene glycol, can be employed, the preferred polyalkylene

glycol materials are those in which one or both of the terminal hydroxy groups have been modified to form ether groups, providing mono- or diether derivatives, or combinations thereof. Thus, the most desirable glycol materials for purposes of the invention are the monoethers and diethers. Particularly satisfactory materials have been found to be the monomethyl ether of polypropylene glycol, the copolymer of ethylene oxide and propylene oxide, monobutyl ether, and the butyl, methyl diether of polypropylene glycol.

The polyalkylene glycol materials employed in the invention composition preferably are substantially hydrophobic materials. It is preferred not to employ those polyalkylene glycol materials that are to any significant extent water miscible and which would accordingly tend to dissolve water at one temperature and crystallize water out at lower temperatures. The molecular weight of the glycol materials can range from about 500 to about 25,000. However, in order to maintain as low a viscosity of the functional fluid as possible at low temperatures, the glycol materials employed should be of low to medium molecular weight, and accordingly should have a molecular weight ranging from about 500 to about 2,000, preferably from about 600 to about 1,200. Also, it is desirable that the polyalkylene glycol component employed be of a type which tends to supercool and to maintain a low viscosity at temperatures down to about -65°F.

However, as previously noted, where the preferred blend of aromatic and aliphatic phosphates is employed, it has been found advantageous to incorporate two or more glycol materials of the types described above, such glycol materials having substantially different molecular weights. Thus, it has been found most desirable to employ a combination of a glycol material, preferably an ether, having a low to medium molecular weight, as defined above, with a high molecular weight glycol material, preferably an ether, the latter material having a molecular weight above about 2,000, generally ranging from about 3,000 to about 25,000.

The ether end groups which preferably are present on the polyalkylene glycol materials are preferably oxyalkyl groups, the alkyl radicals of which can range from 1 to about 8 carbon atoms in length. The longer chain alkyl groups having in excess of 4 carbon atoms, e.g. pentyl, hexyl, heptyl and octyl, are not preferred because polyalkylene glycol ethers of this type have increased viscosity. It is preferred to employ one or more end alkyl groups in the polyalkylene glycol mono- or diether, which have from 1 to 4 carbon atoms. Thus, preferred end alkyl groups are, for example, methyl, ethyl, n-propyl, isopropyl, n-butyl, isobutyl, and the like. It is often desirable that where a diether is employed, one of the end alkyl groups be a methyl or an ethyl radical, while the other end alkyl group of the diether be, for example, a propyl or butyl radical.

The alkylene groups of the polyalkylene glycol material can be an ethylene or propylene group, or mixtures thereof, that is, copolymers containing ethylene and propylene groups. The propylene polymers and ethylene-propylene copolymers, that is, copolymers of ethylene oxide and propylene oxide, are preferred over the ethylene polymers, because of the increased water solubility of the ethylene polymers.

Particularly satisfactory polyalkylene glycol materials for purposes of the invention are the n-butyl methyl, n-butyl ethyl, isobutyl ether, n-propyl ethyl and isopropyl ethyl diethers of polypropylene glycol, the mono-

methyl ether of polypropylene glycol and the copolymer of ethylene oxide and propylene oxide, monobutyl ether.

The preferred polyalkylene glycol materials employed in the invention composition can be produced in known manner from the 1,2-alkylene glycols. Thus, for example, polypropylene glycol materials are prepared by reacting 1,2-propylene oxide and the corresponding alkylene glycol to form poly-1,2-propylene glycol derivatives, and one or both terminal hydroxy groups can be removed to provide the above-noted ether groups, either during or after polymerization. The term "polypropylene glycol" employed in the specification and claims is intended to denote and include the above-noted poly-1,2-propylene glycol derivatives.

As noted above, mixtures of the above polyalkylene glycol materials, e.g. mixtures of polypropylene glycol mono and/or diethers can be used, or mixtures of two copolymers of ethylene oxide and propylene oxide, monobutyl ether, of substantially different molecular weights.

The phosphorus compound, e.g. phosphate ester, is employed in amounts sufficient particularly to provide good fire resistance or flammability characteristics of the functional fluid. Further, the phosphorus compound and glycol material are present in amounts such that the functional fluid composition has a viscosity at -65°F of not greater than about 6,000 cs, preferably not greater than about 4,200 cs, and a viscosity at 210°F of not less than 2.25 cs, preferably not less than about 3.0 cs. Generally, the phosphorus compound, e.g. phosphate ester, or a mixture thereof, is employed in an amount ranging from about 15 to about 90%, preferably about 15 to about 70%, by weight of the functional fluid composition. When employing the above-noted preferred combination of aliphatic and aromatic phosphates, the aliphatic phosphate can be present in an amount ranging from about 10 to about 80%, preferably about 10 to about 60%, and the aromatic phosphate can be present in an amount ranging from about 5 to about 75%, preferably about 5 to about 40%, by weight of the composition. It has often been found desirable to employ a larger amount of the aliphatic phosphate compared to aromatic phosphate, e.g. a ratio of from 3:2 to 8:1 of aliphatic phosphate. However, in some instances a larger amount of aromatic phosphate to aliphatic phosphate can be employed.

The amount of polyalkylene glycol material, e.g. polypropylene glycol monoether or diether, which can be employed separately or in admixture can range from about 10 to about 85%, preferably about 10 to about 70%, by weight of the functional fluid composition. Compositions containing approximately equal weight proportions of the phosphorus compound or phosphorus ester, and polyalkylene glycol material, for example, have been found quite effective. When mixtures of polyalkylene glycol materials are used, a low to medium molecular weight glycol material can be used in an amount ranging from about 8% to about 65%, preferably about 10 to about 40%, and a glycol material of high molecular weight in an amount ranging from about 2 to about 25%, preferably about 4 to about 15%, by weight of the composition. In such mixture of glycol materials, generally the polyalkylene glycol material of low to medium molecular weight is employed in larger amount than the glycol material of high mo-

lecular weight, e.g. in a ratio of 3:2 to 5:1 of the former to the latter.

In any event, the minimum above-noted proportions of at least 15% phosphorus compound, e.g. phosphate ester or a mixture thereof, and at least 10% of the polyalkylene glycol material, or a mixture thereof, by weight, are present in the functional fluid. It will be noted further that when a mixture or combination of phosphate esters is employed, as described above, a single glycol material can be employed, but preferably a mixture thereof, as described above, is used. When only a single glycol material is used, it is preferred to employ the medium to low molecular weight glycol material defined above.

It will be understood that other commonly employed additives such as corrosion inhibitors, oxidation inhibitors, stabilizers, metal deactivators, and the like, such as epoxides, dialkyl sulfides, benzothiazole, phenyl alpha naphthylamine and phenolic oxidation inhibitors, well known as functional fluid additives in the art, can also be incorporated in the functional fluid composition of the invention, in relatively small amounts, if desired.

The following are examples illustrating functional fluid compositions according to the invention, such examples being only illustrative and are not intended as limitative of the invention.

#### EXAMPLE 1

The following composition containing a phosphate ester and a polyalkylene glycol diether was prepared.

| Components                                                                                                | Percent by weight |
|-----------------------------------------------------------------------------------------------------------|-------------------|
| n-butyl-methyl diether of polypropylene glycol (molecular weight, about 700) marketed as "Ucon DLB 62E"   | 37                |
| n-butyl-methyl diether of polypropylene glycol (molecular weight about 1,000) marketed as "Ucon DLB-200E" | 16                |
| tri-n-hexyl phosphate                                                                                     | 47                |
|                                                                                                           | 100               |

The viscosity of the above composition at -65°F, 100°F, and 210°F was measured and the results noted below.

| Temperatures(°F) | Viscosity (centistokes) |
|------------------|-------------------------|
| -65              | 3670                    |
| 100              | 10.1                    |
| 210              | 3.01                    |

#### EXAMPLES 2 and 3

Compositions 2 and 3 noted in Table I below, containing a phosphate ester or esters, and a polypropylene glycol diether or diethers were prepared in accordance with the invention.

The viscosity in centistokes at -65°F and at 210°F, and also the density, of the respective compositions were measured.

The resulting compositions designated Examples 2 and 3 are given in the table below, together with their respective density and viscosities at -65°F and 210°F.

11

| Components                | Examples of Compositions (% by weight) |       |
|---------------------------|----------------------------------------|-------|
|                           | 2                                      | 3     |
| Ucon DLB-200E             | 18                                     | 22.5  |
| Ucon DLB-62E              | 15.5                                   | 19    |
| Di butyl phenyl phosphate | 8                                      | —     |
| Tri-n-hexyl phosphate     | 55                                     | 55    |
| Additives                 | 3.5                                    | 3.5   |
|                           | 100.0                                  | 100.0 |
| <br>Viscosity (cs)        |                                        |       |
| 65°F                      | 2880                                   | 3980  |
| 210°F                     | 2.70                                   | 3.22  |
| Density                   | 0.96                                   | 0.95  |

The term "additives" set forth in the table above includes epoxide stabilizer, 4,4'-dichlorodiphenyl diselenide and triphenyl phosphine, and water.

From the table above, it is seen that the compositions of Examples 2 and 3 containing a phosphate ester, or mixtures thereof, and a polypropylene glycol diether or mixtures thereof, of suitable molecular weight, each have viscosities at  $-65^{\circ}\text{F}$  ranging from 2880 to 3980 cs. and at  $210^{\circ}\text{F}$  ranging from 2.70 to 3.22 cs, and essentially within the preferred viscosities of less than 4200 cs at  $-65^{\circ}\text{F}$  and about 3.0 cs at  $210^{\circ}\text{F}$ , and densities less than 1, and hence are relatively low density fluids, an important economic criterion for use of such fluids in modern large commercial aircraft, so that such compositions are particularly useful as functional or hydraulic fluids in aircraft.

The compositions corresponding to Examples 2 to 3 of the above table also have good fire resistance, and have good thermal and hydrolytic stability.

**EXAMPLE 4**

The following composition containing a combination of aliphatic and aromatic phosphate esters was prepared:

| Components                    | Percent by weight |
|-------------------------------|-------------------|
| Tributyl phosphate            | 49.5%             |
| Santicizer 148                | 24.4%             |
| Ucon LB 285 (a polyglycol)    | 14.1%             |
| Ucon 50HB 5100 (a polyglycol) | 5.6%              |
| A mono epoxide additive       | 6.0%              |
| Bis (phenylthio)-ethane       | 0.4%              |
|                               | 100.0             |

12

Water concentration of the above composition was adjusted to 0.2%, and 0.02% of a perfluorinated alkyl sulfonic acid surfactant was added.

Santicizer 148 is understood to be a mixed alkyl ( $C_8 - C_{13}$ ) diphenyl phosphate.

Ucon LB 285 is understood to be the copolymer of ethylene oxide and propylene oxide, monobutyl ether having a molecular weight of approximately 1,000.

Ucon 50HB 5100 is understood to be the copolymer of ethylene oxide and propylene oxide, monobutyl ether, molecular weight 4,000 - 5,000.

The resulting composition containing a mixture of aliphatic and aromatic phosphates has an improved AIT (autoignition temperature) of about 800°F as compared to an AIT of less than 600°F for the composition of Example 1, containing only an aliphatic phosphate. Further, the low and high temperature viscosity characteristics of the composition of the present example, containing the mixture of low molecular weight and high molecular weight polyalkylene glycol ethers, are similar to the desirable low and high temperature viscosity characteristics of the composition of Example 1.

Rubber compatibility-rubber swell tests for 168 hours immersion of butyl rubber and EPR (ethylene-propylene rubber) in the composition of this example, designated composition 4, and in two different commercial phosphate ester-based low density hydraulic fluid compositions, designated compositions 5 and 6, were carried out and the results are shown in Table II below.

TABLE II

|    |               | Percent rubber swell |      |
|----|---------------|----------------------|------|
|    |               | Butyl                | EPR  |
| 35 | 4             | 7.7                  | 6.8  |
|    | Composition 5 | 14.7                 | 9.1  |
|    | Composition 6 | 15.5                 | 10.7 |

From the above table, it is seen that the amount of  
40 rubber swell on contact of composition 4 according to  
the invention, with butyl rubber and EPR, important  
rubbers widely used in the manufacture of seals for  
aircraft hydraulic systems, is substantially less than in  
the case of the two different phosphate-ester based  
45 hydraulic fluid compositions 5 and 6.

**EXAMPLES 7 – 18**

In Table III below is set forth additional illustrative compositions of the present invention.

TABLE III

|                                                                   | EXAMPLES OF COMPOSITIONS (% by weight) |    |   |    |    |    |    |    |    |    |    |    |
|-------------------------------------------------------------------|----------------------------------------|----|---|----|----|----|----|----|----|----|----|----|
|                                                                   | 7                                      | 8  | 9 | 10 | 11 | 12 | 13 | 14 | 15 | 16 | 17 | 18 |
| di-n-hexyl phenyl phosphate                                       |                                        |    |   |    | 20 |    |    |    |    |    |    |    |
| di-n-butyl phenyl phosphate                                       |                                        |    |   |    |    |    |    |    |    |    |    |    |
| tri-n-butyl phosphate                                             | 65                                     | 30 |   |    | 45 |    |    | 15 |    | 15 |    |    |
| tri-n-hexyl phosphate                                             | 25                                     |    |   | 40 |    | 45 |    |    | 50 | 30 | 40 |    |
| n-butyl diphenyl phosphate                                        | 25                                     |    |   |    | 40 |    |    |    |    |    |    |    |
| n-octyl diphenyl phosphate                                        | 25                                     |    |   |    |    |    | 25 |    |    |    |    |    |
| triphenyl phosphate                                               |                                        |    |   |    |    |    | 25 |    |    |    |    |    |
| di Cresyl phenyl phosphate                                        |                                        |    |   |    |    | 20 |    |    |    |    |    | 15 |
| tricresyl phosphate                                               |                                        |    |   | 15 |    |    |    |    |    | 25 |    | 20 |
| Phenyl-N-methyl-N-n butyl-N'-methyl-N'-n-butyl phosphorodiimidate |                                        |    |   |    |    |    |    | 55 |    |    |    |    |
| Ucon DBL 62E                                                      | 35                                     | 70 |   |    | 25 |    | 45 |    |    |    |    |    |
| Ucon LB 285                                                       | 17                                     |    |   | 45 | 40 |    | 20 |    | 40 | 25 | 22 |    |

TABLE III-continued

|                | EXAMPLES OF COMPOSITIONS (% by weight) |   |   |    |    |    |    |    |    |    |    |    |
|----------------|----------------------------------------|---|---|----|----|----|----|----|----|----|----|----|
|                | 7                                      | 8 | 9 | 10 | 11 | 12 | 13 | 14 | 15 | 16 | 17 | 18 |
| Jeffox OL 2700 |                                        |   |   |    |    | 10 |    |    | 20 |    | 10 |    |
| Ucon 50HB 5100 |                                        | 8 |   |    |    |    | 10 |    |    | 10 | 8  |    |

Jeffox OL 2700 is understood to be a polypropylene glycol monomethyl ether, molecular weight about 3,000.

#### EXAMPLE 19

The following composition was prepared:

| Components         | Parts by weight |
|--------------------|-----------------|
| tributyl phosphate | 495             |
| Santicizer 148     | 244             |
| Ucon LB 285        | 141             |
| Ucon 50HB 5100     | 56              |

The resulting composition had an AIT, low and high temperature viscosity characteristics and rubber compatibility, comparable to the functional fluid composition of Example 4.

From the foregoing, it is seen that in accordance with the invention, functional fluids designed for industrial and marine use, and particularly for use as hydraulic fluids in jet aircraft, are provided in the form of a mixture of a phosphorus compound, preferably an aliphatic phosphate ester containing at least two alkyl groups, and a polyalkylene glycol material, preferably a polypropylene glycol ether, the phosphate ester most desirably being a combination of aliphatic and aromatic phosphates, and the polyalkylene glycol material most desirably being a combination of polyalkylene glycol ethers of low to medium molecular weight, and of high molecular weight, such fluids having requisite viscosity characteristics at temperatures ranging from about -65°F to about 210°F, permitting their use in aircraft hydraulic systems even in the absence of viscosity index improvers, and improved thermal and hydrolytic stability, and which have improved fire resistance and reduced deleterious effect on non-metallic materials, e.g. reduced rubber swell on contact with rubber parts, and also have satisfactory corrosion and pump wear resistance corresponding to conventionally employed phosphate ester base stocks, and desirably low density, with the particular virtue that the resulting invention fluids in which a substantial proportion of phosphorus ester, particularly aliphatic phosphate ester, in conventionally employed phosphorus ester base stocks, is replaced by the abovenoted polyalkylene glycol material, have substantially improved shear stability and substantially reduced cost as compared to the conventional phosphorus ester base stocks.

While I have described particular embodiments of my invention for purposes of illustration, it will be understood that various changes and modifications within the spirit of the invention can be made, and the invention is not to be taken as limited except by the scope of the appended claims.

I claim:

1. A functional fluid composition consisting essentially of (1) a combination of at least two phosphate esters, one of said phosphate esters containing at least two groups selected from the class consisting of alkyl

10 and alkoxyalkyl, and mixtures thereof, and a second of said phosphate esters containing at least two aromatic groups selected from the class consisting of aryl and alkaryl groups, and mixtures thereof, and (2) a combination of at least two polyalkylene glycol ethers containing terminal oxyalkyl groups wherein the alkyl radicals contain from 1 to about 8 carbon atoms, said alkylene groups being selected from the class consisting of ethylene and propylene radicals, one of said polyalkylene glycol ethers having a molecular weight ranging from about 500 to about 2,000, and a second of said polyalkylene glycol ethers having a molecular weight ranging from above 2,000 up to about 25,000, said phosphate esters and said polyalkylene glycol ethers being present in amounts such that said composition has a viscosity at -65°F of not greater than about 6,000 centistokes, and a viscosity at 210°F of not less than 2.25 centistokes.

2. A functional fluid composition as defined in claim 1, said phosphate esters and said polyalkylene glycol ethers being present in amounts such that said composition has a viscosity at -65°F not greater than about 4,200 centistokes and a viscosity at 210°F not less than about 3.0 centistokes.

3. A functional fluid composition as defined in claim 1, said one phosphate ester being present in an amount ranging from about 10 to about 80%, and said second phosphate ester being present in an amount ranging from about 5 to about 75%, said one polyalkylene glycol ether being present in an amount ranging from about 8 to about 65%, and said second polyalkylene glycol ether being present in an amount ranging from about 2 to about 25%, by weight of said composition.

4. A functional fluid composition as defined in claim 3, said one phosphate ester having the general formula:



50 where  $R_1$  and  $R_2$  are each a member selected from the group consisting of alkyl of from about 3 to about 10 carbon atoms, and alkoxyalkyl having from about 3 to about 8 carbon atoms, and  $R_3$  is a member selected from the group consisting of alkyl and alkoxyalkyl, as above defined, aryl and alkaryl, containing from 6 to about 8 carbon atoms, said second phosphate ester having the general formula:



65 where  $R_4$  and  $R_5$  are each a member selected from the group consisting of aryl and alkaryl, containing from 6 to about 8 carbon atoms, and  $R_6$  is a member selected from the group consisting of aryl and alkaryl, containing from 6 to about 8 carbon atoms, alkyl of from about

3 to about 20 carbon atoms, and alkoxyalkyl having from about 3 to about 8 carbon atoms.

5. A functional composition as defined in claim 4, wherein said one phosphate ester is selected from the group consisting of dialkyl aryl and trialkyl phosphates, and said second phosphate ester is selected from the group consisting of triaryl and alkyl diaryl phosphates.

6. A functional fluid composition as defined in claim 3, said polyalkylene glycol ethers selected from the group consisting of a polypropylene glycol mono- or diether, and a mono- or diether of an ethylene-propylene copolymer, said mono- or diethers having at least one terminal oxyalkyl group wherein the alkyl radicals contain from 1 to about 4 carbon atoms.

7. A functional fluid composition as defined in claim 4, said polyalkylene glycol ethers selected from the group consisting of a polypropylene glycol mono- or diether, and a mono- or diether of an ethylene-propylene copolymer, said mono- or diethers having at least one terminal oxyalkyl groups wherein the alkyl radicals contain from 1 to about 4 carbon atoms.

8. A functional fluid composition as defined in claim 7, said one polyalkylene glycol ether having a molecular weight ranging from about 600 to about 1,200, and said polyalkylene glycol ether having a molecular weight ranging from about 3,000 to about 25,000.

9. A functional composition as defined in claim 8, wherein said one phosphate ester is selected from the group consisting of dialkyl aryl and trialkyl phosphates, and said second phosphate ester is selected from the group consisting of triaryl and alkyl diaryl phosphates.

10. A functional fluid composition as defined in claim 9, said one phosphate ester being present in an amount ranging from about 10 to about 60%, and said second phosphate ester being present in an amount ranging from about 5 to about 40%, said one polyalkyl-

ene glycol ether being present in an amount ranging from about 10 to about 40%, and said second polyalkylene glycol ether being present in an amount ranging from about 4 to about 15%, by weight of said composition.

11. A functional fluid composition as defined in claim 7, said one phosphate ester being selected from the group consisting of tributyl phosphate, dibutyl phenyl phosphate and tri-n-hexyl phosphate, and said second phosphate ester being selected from the group consisting of tricresyl phosphate, butyl diphenyl phosphate and tridecyl diphenyl phosphate.

12. A functional fluid composition as defined in claim 10, said one phosphate ester being selected from the group consisting of tributyl phosphate, dibutyl phenyl phosphate and tri-n-hexyl phosphate, and said second phosphate ester being selected from the group consisting of tricresyl phosphate, butyl diphenyl phosphate and tridecyl and diphenyl phosphate.

13. A functional fluid composition as defined in claim 11, said polyalkylene glycol ethers being selected from the group consisting of the n-butyl methyl diether of polypropylene glycol, the monomethyl ether of polypropylene glycol, and the copolymer of ethylene oxide and propylene oxide, monobutyl ether.

14. A functional fluid composition as defined in claim 12, said polyalkylene glycol ethers being selected from the group consisting of the n-butyl methyl diether of polypropylene glycol, the monomethyl ether of polypropylene glycol, and the copolymer of ethylene oxide and propylene oxide, monobutyl ether.

15. A functional fluid composition as defined in claim 14, wherein both said one and said second polyalkylene glycol ethers are each a copolymer of ethylene oxide and propylene oxide, monobutyl ether.

\*\* \* \* \* \*

16. A functional fluid composition as defined in claim 15, wherein both said one and said second polyalkylene glycol ethers are each a copolymer of ethylene oxide and propylene oxide, monobutyl ether.